

# UNITED STATES PATENT OFFICE.

HENRY SUTTON, OF BALLARAT, VICTORIA.

## PROCESS OF CONVERTING A PHOTOGRAPHIC IMAGE ON A GELATINE SURFACE INTO A RELIEF OR INTAGLIO.

SPECIFICATION forming part of Letters Patent No. 381,091, dated April 10, 1888.

Application filed November 9, 1887. Serial No. 254,698. (No specimens.)

*To all whom it may concern:*

Be it known that I, HENRY SUTTON, a subject of the Queen of Great Britain, residing at Ballarat, in the British Colony of Victoria, 5 music-seller, have invented an Improved Process of Converting a Photographic Image on a Gelatine Surface into a Relief or Intaglio Printing-Surface; and I do hereby declare that the following is a full, clear, and exact description 10 of the invention, which will enable others skilled in the art to which it appertains to make and use the same.

It is well known that relief and intaglio printing-surfaces can be produced from photographs; but in practice these have been principally confined to the production of linear work on account of the difficulty of faithfully representing the delicate shades of what are known as the "half-tones." When such half-tones have been represented it has been due to the exercise of very great manual skill, and when produced it requires very great care and ability on the part of the printer to produce a satisfactory representation on paper.

It is well known that the half-tones of photographs may be "broken up" by dot, stipple, line hatch, grain, or other pattern.

I know of no method by which a photographic image on a gelatine surface can be automatically converted into a relief or intaglio printing-surface.

Now, this invention is designed for the especial purpose of automatically converting a photographic image on a gelatine surface 35 into a relief or intaglio printing-surface which will faithfully represent the delicate lights and shades or half-tones, said printing-surface being of such a kind that an ordinary printer with ordinary appliances can without difficulty 40 utilize it for printing purposes.

In carrying out my process, I take an ordinary sensitized gelatine plate bearing a photograph broken up by any pattern or grain, as before described, and I immerse it in water, 45 the temperature of which must be below that at which the particular gelatine used will melt or dissolve. Here I allow it to remain until all the gelatine swells by absorption of water; but the extent to which this is allowed must 50 be determined by the character of the picture

and the judgment of the operator. After removing the plate from this bath I remove the free water from its surface, preferably by a slight rinse in alcohol or spirits of wine. I then subject this plate to a gradually-increasing temperature until it reaches about that at which the particular gelatine used begins to melt, and I continue this heat until all or nearly all the water or moisture is driven off. The result of this is that those portions of the gelatine which are unaffected by the action of light and which are freely absorbent of water melt and are drawn by capillary attraction under the unmelted portions, forcing the latter up in relief, the dots, stippling, lines, grains, hatch, 65 or other pattern by which the photographic image is broken up being graduated in size and form in precise proportion to the action of light, and of light and development, on such photographic image. This completes my process. 70

If the photographic image on the plate heated be a "negative" the printing-surface produced will be in intaglio; if it be a "positive" the printing-surface will be in relief. 75

If the gelatine be on a sufficiently thick sheet of glass, or on wood or metal or other hard material, it may be used direct in a typographic press, or if on metal or other suitable surface it may be used direct in the copper-plate press; 80 but if it be on the ordinary thickness of glass, electrotypes or stereotypes must be used for the copper-plate press. I find that electrotypes and stereotypes may be made from my printing-surfaces in the same way, and much 85 more easily and quickly than from ordinary engravings, inasmuch as I can electrotype direct on my printing-surfaces, thus saving the usual "wax squeeze," and I can cast stereotype metal direct on my printing-surfaces 90 without the intervention of the paper or plaster molds used in stereotyping.

In actual practice, I have taken an ordinary gelatine dry-plate (Fry's transparency make) and have impressed an image thereon by the 95 action of light, such image having its surface diversified or broken up by the ordinary wire-gauze pattern, and have then developed and fixed the image in the usual way. I have then immersed this for five minutes in water of the 100

temperature of 80° Fahrenheit, and have then removed the free water by dipping the plate in a bath of spirits of wine for ten seconds, and have then removed the plate and fanned 5 the spirits of wine dry from its surface. I have then placed it on a copper plate supported on feet or legs, and heated it by means of a Bunsen gas-burner until it became about the temperature of 212° Fahrenheit. This heat I have 10 continued for two minutes, when I have found my object accomplished.

I do not confine myself to any particular uses to which my printing-surfaces may be applied, and I wish it to be distinctly understood 15 that I do not claim the production of photographic pictures on gelatine plates broken up or diversified by dot, stipple, grain, or pattern of any kind, nor to the immersion of such plates in water for the purpose of causing the unaffected gelatine to swell and rise into relief, as I am aware that all this has been done before; but 20

What I do claim as of my invention is—  
The herein-described method of converting a photographic image on a gelatine surface 25 into a relief or intaglio printing-surface, which consists in immersing the plate bearing the photographic image in water of a temperature below that of the melting-point of the unexposed parts of the gelatine, in order to swell 30 the same by absorption, then taking out the plate and removing the free water from the surface thereof, then exposing the plate to a degree of heat at which the unexposed parts of the gelatine will begin to melt until the wa- 35 ter-absorbed gelatine has been dissolved, substantially as described.

HENRY SUTTON.

Witnesses:

EDWARD WATERS,  
WALTER CHARLES HART.